

## UNITED STATES PATENT OFFICE

2,029,088

## PROCESS FOR TANNING

Harold G. Turley, Moorestown, N. J., and Ian C. Somerville, Fox Chase, Pa., assignors to Röhm & Haas Company, Philadelphia, Pa.

No Drawing. Application May 12, 1934,  
Serial No. 725,314

13 Claims. (Cl. 149—5)

This invention relates generally to an improved process for tanning raw hides or skins and more particularly for the purpose of making white leather.

5 Raw skins or hides may be converted into leather in several different ways, depending on the type of leather desired. In all cases the skins are first treated to remove the hair. This may be done in a variety of different ways, using

10 lime, sodium sulfide, etc. During this process the leather-producing fibers are rendered soft and supple and satisfactory for making leather. The skins so prepared are then tanned, and this process

15 may be carried out in numerous different ways. For instance, the tanning may be accomplished by the use of extracts of the vegetable tannins, in which case an excellent leather, generally of a brownish color is produced. Such leather, however, is not resistant to hot water.

20 The second method of tanning consists in the use of mineral salts, particularly those of aluminum and chromium. The aluminum salts may yield a white leather which, however, is not generally resistant to washing with cold water nor

25 to a short treatment with hot water. It is usually a thin flat leather suitable for making gloves but less satisfactory for "full" "round" shoe leathers. When chromium salts are used a leather is obtained which is resistant to hot water and consequently this process is in very wide use, particularly on light weight skins. On the other hand, such leather always has a blue or greenish blue color so that it is very difficult to produce a good white color on this stock.

30 A third method of tanning which has found a limited use consists in the application of aldehydes, particularly of formaldehyde. The leather produced by this method is white and does not break down on treatment with hot water. However, it is of a thin flat character, absorbs water instantly and subsequently dries out so hard that it is unsuitable for many purposes.

35 Many materials prepared synthetically have been tried as tanning agents and are capable of producing good leathers. However, such leathers have the same drawback as those made with vegetable tannins, namely, lack of resistance to hot water.

40 We have found that a good white leather having high resistance to both hot and cold water may be made by certain combinations of steps in the tanning process. It is an object of this invention to prepare a leather which is of unusually good quality with respect to color, feel, fullness, 45 resistance to hot and cold water, and which after

treatment with hot water dries out soft and supple. It is a further object of this invention to prepare a white leather which does not discolor in light, which is free from any trace of a blue or brownish color, and which is white throughout. 5 It is another object of this invention to prepare a leather on which delicate shades and bright colors may be produced. It is a further object to prepare a suede leather which has exceptionally good color and water resistance and a very 10 smooth nap. Other objects will appear hereinafter.

In carrying out our invention, the skins prepared for tanning are adjusted to a definite degree of acidity and a combination tannage is 15 built up in a series of steps, each of which contributes its peculiar quality to the finished leather. In this way a leather is obtained which is surprisingly superior to that made according to any one of the individual steps of this particular 20 combination tannage. Briefly, this is accomplished by applying to the skins, at a definite degree of acidity either successively or simultaneously, a suitable aldehyde, a salt of aluminum of a definite basicity and a synthetic tanning material. These tanning agents may be added to the leather successively in any order, or two may be used simultaneously, followed by the third, or all three may be used at the same time. Leather tanned in this way may be fatliquored and finished in any suitable manner. The following is 25 our preferred method of carrying out this invention:

The skins are treated in the customary way up to the pickled condition. They are then de- 35 pickled in a drum in a weak solution of common salt until they show a pH of approximately 4.5. To this same drum is then added 10% by weight of a 37% solution of formaldehyde, whereupon the drum is run for five hours and allowed to stand overnight. The percentages of materials added are based on the pickled weight of the skins. An unusual feature of our invention is the discovery that the formaldehyde tannage may be carried out at a pH in the vicinity of the isoelectric point 40 of the hide protein. On the following day, a solution of alum of the proper basicity and concentration is added. The drum is run for five hours and again allowed to stand overnight. The alum solution contains from 1.25 to 2.25% of aluminum 45 oxide in the form of a 40% basic aluminum sulphate, the basicity being calculated on the Schoregger scale. Such a solution can be conveniently prepared by dissolving the proper amount of commercial aluminum sulphate, free 50

of iron salts, in water and adding the calculated amount of a weak alkali, such as sodium bicarbonate, borax or soda ash. On the third day, the liquor is drawn off and the skins washed thoroughly for one-half hour to an hour until free of salts. 10% of a commercial synthetic tanning material, which has been adjusted to a pH of 4.5, is then added to the skins in a convenient quantity of water and the drum is run until all 5 of the tanning agent has been removed from the liquor. The skins are then washed thoroughly and fatliquored with a suitable oil in the usual way. We have found that most of the commercial sulphonated oils recommended for use on 10 white leather are suitable for the leather produced by our process. The skins are then hung up and allowed to dry slowly. The resulting leather is white throughout and very resistant to wetting but can be moistened back slowly. These skins 15 may be staked and finished in any desired manner. The leather obtained by this process is pure white and may be used as such or dyed to give any desired color. It is particularly advantageous as a base for pastel shades. The skins may 20 be dyed by any of the standard methods, using acid, direct or basic dyes, following which they may be fatliquored and finished as usual.

Our invention may be illustrated by the following examples, but it is not limited to the specific details since the invention may be otherwise practiced within the scope of the appended 30 claims:

*Example 1.*—100 lbs. of pickled kidskins are placed in a small drum with 200 lbs. water and 35 10 lbs. common salt. Bicarbonate of soda is added in successive small amounts and the drum run until the skins show a uniform pH of 4.5. To the skins in the same liquor is added 10 lbs. of formaldehyde (37%), the drum run 5 hours and then shut down overnight. Next day the drum is run 1 hour, then 100 lbs. of a solution containing 8 lbs. of sulfate of alumina (14H<sub>2</sub>O) and 2 1/4 lbs. sodium bicarbonate is added. The drum is run 5 hours and then shut down overnight. 40 Next day, the drum is run 1 hour, the liquor drained off, and the skins washed for 1/2 hour. 200 lbs. water containing 10 lbs. of a synthetic tanning material, made by condensing phenol sulphonic acid with formaldehyde is then 45 added. This solution is adjusted to a pH of 4.5 before putting it in the drum. The drum is run for 1 hour, the liquor drained off, the skins washed for 1/2 hour, fatliquored with 5 lbs. of sulfonated neat's-foot oil and horsed up overnight. Next day, they are shaved if desired, and 50 hung to dry in a cool room, after which they are processed according to the methods in general use for the treatment of skins which have been crusted, to yield a soft white leather of good grain and excellent fullness, which is not readily wet with cold water and which will not shrink when treated with water as hot as 180° F.

*Example 2.*—100 lbs. of pickled sheepskins are placed in a small drum with 100 lbs. of water and 65 10 lbs. common salt. Soda ash is added in successive small amounts and the drum run until the skins show a uniform pH of 4.75. To the skins in the same liquor, 10 lbs. of 37% formaldehyde solution is then added, the drum run for 5 hours and then shut down overnight. Next day, the drum is run 1 hour, 100 lbs. water is added, and a dry mixture of 15 lbs. sulfate of alumina (14H<sub>2</sub>O) and 12 lbs. borax thrown in. The drum is run 5 hours and then shut down overnight. 70 Next day the drum is run 1 hour, the liquor

drained off, and the skins washed for 1/2 hour. 200 lbs. water containing 18 lbs. of a synthetic tanning material prepared by the sulfonation of 4,4'-dihydroxydiphenyldimethylmethane is added, the solution being adjusted to a pH of 4.5 5 prior to putting in the drum. The drum is run 1 1/2 hours, the liquor drained off, the skins washed for 1/2 hour, fatliquored with 10 lbs. of sulfonated cocoanut oil and horsed up overnight. Next day they are tacked in the wet state, dried 10 in a cool room, and finished up in the customary way.

*Example 3.*—100 lbs. of pickled calfskins are placed in a small drum with 200 lbs. water and 10 lbs. of common salt. Bicarbonate of soda is 15 added in successive small amounts until the skins show a uniform pH of 5.0. To the skins in the same liquor is added a dry mixture of 4 lbs. water-soluble paraformaldehyde, 15 lbs. sulfate of alumina (14H<sub>2</sub>O), and 12 lbs. borax, the drum 20 run for 5 hours and then shut down overnight. The drum is again run for 5 hours the following day and shut down overnight. On the third day the drum is run for 1 hour, the liquor drained off and the skins washed for 1/2 hour. 15 lbs. of a 25 synthetic tanning material prepared by condensing naphthalene sulfonic acid with formaldehyde and adjusted to pH 4.5 is then added. The drum is run for 1 hour, the liquor drained off, the skins washed for 1/4 hour and then horsed up 30 overnight. Next day, they are set out, shaved, washed for 1/4 hour and fatliquored with 3 lbs. of a sulfonated blend of neat's-foot, cocoanut, and sperm oils. When this oil is almost all taken up by the skins, 1 lb. of titanium oxide dispersed 35 in warm water is added and the drum run 1/2 hour longer. The skins are then hung to dry in a cool room, and processed later in the customary way.

*Example 4.*—100 lbs. of pickled calfskins are 40 placed in a small drum and 200 lbs. of water and 10 lbs. common salt. Borax is added in successive small amounts and the drum run until the skins show a uniform pH of 4.25 to 4.5. This liquor is drained and 200 lbs. water added, 7 lbs. 45 of a synthetic tanning material prepared by coupling benzidine disulfonic acid with a substituted aromatic sulfonyl chloride substantially as described in U. S. Patent #1,938,022 is added. The drum is run 1 hour, 10 lbs. of formaldehyde (37% solution) added to the same liquor, the drum run 5 hours, and shut down overnight. Next day the drum is run 1 hour and 100 lbs. 50 of a solution containing 15 lbs. sulfate of alumina (14H<sub>2</sub>O) and 3 lbs. of soda ash added. The drum is run 5 hours and shut down overnight. It is run 1 hour next day, the liquor drained off, the skins washed for 1/2 hour, then fatliquored with 4 lbs. of sulfonated cocoanut oil, and horsed up 55 overnight. Next day, they are set out, shaved, hung up and allowed to dry. The crusted skins are wet back slowly, staked and tacked, then buffed and brushed on the flesh side to give a white suede leather of excellent whiteness and possessing a fine nap.

*Example 5.*—100 lbs. of pickled calfskins are placed in a small drum with 200 lbs. water and 10 lbs. common salt. Bicarbonate of soda is added in successive small amounts and the drum run until the skins show a uniform pH of 4.5. To the same liquor is added 10 lbs. formaldehyde (37% solution), 14 lbs. of sulfate of alumina (14H<sub>2</sub>O), 11 lbs. borax, and 15 lbs. of a synthetic tanning material prepared by condensing naphthalene sulfonic acid with formaldehyde in the 75

presence of salicylic acid, the complete solution being adjusted to a pH of 4.5. The drum is run intermittently for 48 hours and the skins horsed up 24 hours. They are then set out, shaved, washed for  $\frac{1}{2}$  hour, and fatliquored with 4 lbs. of sulfonated olive oil. When the oil is almost all taken up by the skins, 5 lbs. of English colloidal clay dispersed in warm water is added to the drum, and this is run  $\frac{1}{2}$  hour longer. The skins are then hung up, allowed to dry in a cool room and processed later in the ordinary way.

Example 6.—100 lbs. of pickled calfskins are processed in exactly the same way as the sheepskins in Example 2, except that 10 lbs. of synthetic tanning material prepared by sulfonation of the liquid resin formed by condensation of phenol with acetaldehyde, is added in place of the synthetic material used in Example 2.

Example 7.—100 lbs. of pickled calfskins are processed in exactly the same way as in Example 6, except that 8 lbs. of a synthetic tanning material prepared by condensing the sulfonation product of tertiary amyl phenol with formaldehyde in presence of salicylic acid and/or thiourea is added in place of the synthetic material used in Example 6.

Example 8.—100 lbs. of pickled calfskins are placed in a small drum with 100 lbs. water and 10 lbs. common salt. Soda ash is added in successive small amounts and the drum run until the skins show a uniform pH of 4.75. To the skins in the same liquor is added 10 lbs. of formaldehyde (37% solution), the drum run 5 hours and then shut down overnight. Next day, 100 lbs. of a solution containing 23 lbs. potash alum and 5 lbs. bicarbonate of soda is added, the drum run 5 hours and then shut down overnight. Next day, the skins are washed thoroughly and the tanning is completed by application of a synthetic tanning material as described in Examples 1, 2, or 3.

Example 9.—200 lbs. of side leather in the pickled condition are placed in a drum with 400 lbs. water and 20 lbs. common salt. Bicarbonate of soda is added in successive small portions, drumming until the hides show a uniform pH of 4.75. 24 lbs. of formaldehyde, (37% solution), is added and the drum run for 5 hours. 30 lbs. of sulfate of alumina ( $14\text{H}_2\text{O}$ ) and 24 lbs. borax are then thrown in, and the drum run intermittently for 20 hours. The skins are horsed up for two days, set out and shaved, washed  $\frac{1}{2}$  hour, 20 lbs. of a synthetic tanning material as given in Example 4, adjusted to a pH of 4.5 is then added, the drum is run  $1\frac{1}{2}$  hours, drained, and the skins washed  $\frac{1}{2}$  hour, and fatliquored with 6% of an oil made by sulfonation of a blend of neat's-foot, castor and cocoanut oils. The skins are horsed up overnight and crusted. After wetting back slowly, they are staked out and tacked, then buffed on the grain side to give a soft white imitation buckskin of excellent feel which is resistant to wetting with cold water and will not shrink when treated with water at  $180^{\circ}\text{ F}$ .

Example 10.—300 lbs. of pickled calfskins are depickled and tanned in the same manner as in Example 5. After the skins have been horsed up for 24 hours, they are divided into smaller lots and colored in several ways. (a) 100 lbs. are placed in 100 lbs. water at  $120^{\circ}\text{ F}$ . and 1 lb. of Acid Leather Brown ER is added. The drum is run  $\frac{1}{2}$  hour, the skins rinsed off with warm water and fatliquored in the normal way. (b) 100 lbs. are placed in 100 lbs. water at  $120^{\circ}\text{ F}$ . and 1 lb. of Direct Fast Brown TSL is added. The drum is

run  $\frac{1}{2}$  hour, 1 lb. formic acid is added, and drumming is continued for  $\frac{1}{2}$  hour. The skins are washed, fatliquored and finished up in the normal way. (c) 100 lbs. are placed in 100 lbs. water at  $120^{\circ}\text{ F}$ . and  $\frac{1}{2}$  lb. of Basic Black A. conc. is added. The drum is run  $\frac{1}{2}$  hour, the skins rinsed off and fatliquored in the normal way. In this way a rich full black color is secured which provides a pleasing contrast to the white leather obtained when no color is applied, and moreover shows a pure white cut.

Example 11.—100 lbs. of pickled sheepskins are placed in a small drum with 200 lbs. water and 20 lbs. common salt. Bicarbonate of soda is added in successive small amounts and the drum run until the skins show a uniform pH of  $4\frac{3}{4}$ . To the skins in the same liquor is added 9 lbs. of crotonaldehyde, and the drum run intermittently for 24 hours. A mixture of 10 lbs. iron free aluminum sulfate and 8 lbs. borax is added and the drum run 5 hours, then shut down overnight. The skins are thoroughly washed and the tanning then completed by application of a synthetic tanning material as in Example 1. In this way, a soft leather of excellent feel and a creamy white color is obtained.

Example 12.—100 pounds of pickled and degreased cape skins are placed in a small drum with 100 pounds of water and 10 pounds of salt. Bicarbonate of soda is added in small amounts and the drum run until the skins show a uniform pH of  $4\frac{1}{2}$ . To the skins in the same liquor, 10 pounds of 37% formaldehyde is then added and the drum run for 5 hours. Then 100 pounds of water containing 2 pounds of aluminum sulphate and 1 pound of borax is added and the drumming continued for 5 hours and then shut down overnight. Next day the drum is run for 1 hour, liquor drained off, and the skins washed for  $\frac{1}{2}$  hour. 200 pounds of water containing 5 pounds of a synthetic tanning material prepared by the sulfonation of 4,4'-dihydroxydiphenyldimethylmethane is added. The drum is run  $1\frac{1}{2}$  hours, the liquor drained off, the skins washed for  $\frac{1}{4}$  hour, fatliquored with 15 pounds of a sulfonated cocoanut oil, and horsed up overnight. Next day they are allowed to crust out. On staking and finishing in the customary way, a soft, white glove leather is obtained.

Many modifications and variations within the spirit of this invention will suggest themselves to those versed in the art. For instance, the nature of the raw stock used may be varied from those specifically mentioned in the examples.

A complete tanning can also be secured, if desired, by reducing the amount of material used in any one step and compensating by an increase in the amount of the material used in either of the other steps. For instance, the formaldehyde may be reduced by  $\frac{1}{2}$  and the amount of alum or synthetic tanning material doubled. This is true irrespective of whether the process is carried out in a single step, two steps or three steps. It will therefore be readily understood that no precise limits can be set for the quantity of any one of the reagents but a balance must be maintained among them, based approximately on the amounts specified in the examples.

These processes are carried out at temperatures commonly used in tannery practice. It is convenient to start with liquors at about  $80^{\circ}\text{ F}$ . since this can be maintained rather readily at any season of the year. Formaldehyde tanning occurs more readily the higher the temperature but it is not good practice to exceed  $80^{\circ}\text{ F}$ . in the early

stages, or 110° F. in the later stages until after all the formaldehyde has been fixed in the skins. Although we prefer, in making a smooth grained leather, to apply the formaldehyde under the acid conditions described, yet, for some purposes, it is naturally obvious that the formaldehyde tannage can be carried out as is more customary; viz., in an alkaline bath. The formaldehyde may be replaced by other suitable aldehydes, such as croton aldehyde. The alum can be adjusted to the desired basicity by various alkalies. It is preferably applied at the basicity of 40 on the Schorlemmer scale. However, this may be reduced to a rather lower figure, say to 35, and may also be increased somewhat, say to 45. In the latter case, however, a complication is introduced owing to the low solubility of an alum of much higher basicity than 40, when used at the dilutions normally employed in tanning. The amount of synthetic tanning material can be very greatly increased if desired even up to ten times the amount given in the examples. In such cases a softer and more mellow leather is obtained.

This process of tanning may be used to produce leathers of widely varying characteristics. As examples may be mentioned, side leather, calf-skin, buckskin (genuine and imitation), suede, kid-skin, sheepskin, glove, reptile, welting leather, etc. While primarily designed to make white leather which will have no trace of blue cast, and will show a white cut all the way through, this process is capable of use as a standard method of making leather which can be colored to any shade desired. However, its special merit lies in the fact that delicate shades of pure colors can be obtained because the leather has no color before applying the dyestuffs.

The leathers produced by this process are distinctly different from those produced by other processes. In the first place, a white leather is obtained which is different from the darker colored leathers obtained by the use of vegetable and chrome tans. It has a considerably greater resistance to water than leathers made by the formaldehyde process, alum process or a combination of the two.

We claim:

1. The step in the process of tanning which comprises treating skins and hides with an aldehyde capable of reacting with the hide protein, a salt of aluminum and a synthetic organic tanning material.

2. The step in the process of tanning which comprises treating skins and hides which have been adjusted to a pH of 4.25 to 5.0 with an aldehyde capable of reacting with the hide protein, a salt of aluminum and a synthetic organic tanning material.

3. The step in the process of tanning which comprises treating skins and hides which have been adjusted to a pH of 4.25 to 5.0 with an aldehyde capable of reacting with the hide protein, a salt of aluminum and a synthetic organic tanning material, these agents being applied to the skin in any order.

4. The step in the process of tanning which comprises treating skins and hides which have

been adjusted to a pH of 4.25 to 5.0 with an aldehyde capable of reacting with the hide protein, a basic salt of aluminum and a synthetic organic tanning material.

5. The step in the process of tanning which comprises treating skins and hides which have been adjusted to a pH of 4.25 to 5.0 successively with formaldehyde, a salt of aluminum of about 40% basicity, and a synthetic organic tanning material, these agents being applied to the skin in any order.

6. The step in the process of tanning which comprises treating skins and hides which have been adjusted to a pH of 4.25 to 5.0 simultaneously with formaldehyde, a salt of aluminum of about 40% basicity, and a synthetic organic tanning material.

7. The step in the process of tanning which comprises treating skins and hides successively, (A) with a mixture of two of the group consisting of formaldehyde, a basic aluminum salt and a synthetic organic tanning material and (B) with the third member of the group.

8. The step in the process of tanning which comprises treating skins and hides which have been adjusted to a pH of 4.25 to 5.0 successively, (A) with a mixture of two of the group consisting of formaldehyde, a basic aluminum salt and a synthetic organic tanning material and (B) with the third member of the group.

9. The step in the process of tanning which comprises treating skins and hides which have been adjusted to a pH of 4.25 to 5.0 successively, (A) with a mixture of two of the group consisting of formaldehyde, a basic aluminum salt and a synthetic organic tanning material and (B) with the third member of the group, the two treatments taking place in either order.

10. The step in the process of tanning which comprises treating skins and hides which have been adjusted to a pH of 4.25 to 5.0 successively with croton aldehyde, a basic salt of aluminum and a synthetic organic tanning material, these agents being applied to the skin in any order.

11. The step in the process of tanning which comprises treating skins and hides which have been adjusted to a pH of 4.25 to 5.0 simultaneously with croton aldehyde, a basic salt of aluminum and a synthetic organic tanning material.

12. The step in the process of tanning which comprises treating skins and hides which have been adjusted to a pH of 4.25 to 5.0 successively with (A) a mixture of two of the group consisting of croton aldehyde, a basic salt of aluminum and a synthetic organic tanning material and (B) with the third member of the group, the two treatments taking place in either order.

13. The step in the process of tanning which comprises treating skins and hides which have been adjusted to a pH of 4.25 to 5.0 successively with (A) a mixture of formaldehyde and a basic salt of aluminum, and with (B) a synthetic organic tanning material, the two steps taking place in either order.

HAROLD G. TURLEY. 65  
IAN C. SOMERVILLE.